

# United States Patent [19]

Sato et al.

[11] 3,925,084

[45] Dec. 9, 1975

[54] FOGGED, DIRECT-POSITIVE SILVER HALIDE EMULSION CONTAINING A CYANINE DYE HAVING A PYRAZOLO[1,5-a]BENZIMIDAZOLE NUCLEUS

[75] Inventors: **Akira Sato; Keisuke Shiba; Masanao Hinata**, all of Kanagawa, Japan

[73] Assignee: **Fuji Photofilm Co., Ltd.**, Minami-ashigara, Japan

[22] Filed: **Apr. 16, 1973**

[21] Appl. No.: **351,386**

[30] **Foreign Application Priority Data**

Apr. 14, 1972 Japan ..... 47-37445

[52] U.S. Cl. ..... **96/101; 96/107; 96/108;**  
96/130; 260/240 E

[51] Int. Cl.<sup>2</sup> ..... **G03C 1/36; G03C 1/28**

[58] **Field of Search** ..... 96/101, 107-108,  
96/130; 260/240 E

[56]

**References Cited**

UNITED STATES PATENTS

3,758,309 9/1973 Bailey et al. .... 96/136

*Primary Examiner*—Won H. Louie, Jr.

*Attorney, Agent, or Firm*—Sughrue, Rothwell, Mion, Zinn & Macpeak

[57]

**ABSTRACT**

Direct positive silver halide emulsions sensitized by a cyanine dye in which the carbon atom at the 3-position of the pyrazolo[1,5-a]benzimidazole nucleus is joined by a methine chain to the 2-position or the 4-position of the cyanine heterocyclic nucleus, linkage to the 4-position being, however, only when the cyanine heterocyclic nucleus is a quinoline nucleus or a pyridine nucleus.

**29 Claims, No Drawings**

**FOGGED, DIRECT-POSITIVE SILVER HALIDE  
EMULSION CONTAINING A CYANINE DYE  
HAVING A PYRAZOLO[1,5-a]BENZIMIDAZOLE  
NUCLEUS**

**BACKGROUND OF THE INVENTION**

1. Field of the Invention

This invention relates to photographic silver halide emulsions, more particularly, it relates to a direct positive silver halide emulsion sensitized by a dye having a novel pyrazolo[1,5-a]benzimidazole nucleus.

2. Description of the Prior Art

When a silver halide photographic material is exposed to light containing wave lengths in the sensitive wave length region of the photographic material and then developed, the blackened density thereof increases with increased exposure amounts up to a maximum value, but if the exposure amount further increases the blackened density again reduces. This phenomenon is generally called "solarization".

Also, in a silver halide photographic material having a silver halide emulsion layer which has been optically or chemically fogged during the production of the silver halide emulsion, a reversal effect similar to that in solarization, namely the phenomenon that the blackened density again decreases as the exposure increases, is observed. By utilizing such a phenomena, positive images can be obtained.

The term "direct positive silver halide emulsion" in this specification means a silver halide emulsion prepared such that it directly forms a positive image after ordinary exposure to light, i.e., positive light image development.

As sensitizers for ordinary negative silver halide emulsions there are known many dyes such as monomethinecyanine dyes, trimethinecyanine dyes, merocyanine dyes and rhodacyanine dyes. However, the use of these dyes for the sensitization of direct positive silver halide emulsions is frequently accompanied with disadvantages, for instance, softening or flattening of characteristic curves and re-reversal (the phenomenon that with an increase in the exposure amount the blackened density decreases and then the blackened density increases again).

Also, dyes conventionally known as sensitizers for direct positive silver halide emulsions frequently have faults such as leaving color stains after processing of photographic silver halide materials containing them. The formation of such color stains is particularly inconvenient for color photographic papers. When such dyes are used as sensitizers high whiteness is not obtained in black and white photographic papers and further true color reproduction cannot be obtained in color photographic papers. Furthermore, the formation of such color stains is particularly undesirable in hard or high contrast photographic materials used for lithographic films, X-ray photographic films, duplication films for microphotographs, etc.

The dyes used for the sensitization of direct positive silver halide emulsions should not exhibit the above faults and further should not reduce the maximum density of the images formed.

**SUMMARY OF THE INVENTION**

An object of this invention is, therefore, to provide a direct positive silver halide emulsion of high sensitivity, desired maximum image density and further giving substantially no color stains.

As the result of intensive investigations to reach the above-indicated object, the inventors succeeded in reaching the present invention.

That is to say, the invention provides a direct positive silver halide emulsion containing at least one cyanine dye in which the carbon atom of the 3-position of the pyrazolo[1,5-a]benzimidazole nucleus is joined to the 2-position or the 4-position of the cyanine heterocyclic nucleus by a methine chain, joining to the 4-position being, however, only when the cyanine heterocyclic nucleus is a quinoline nucleus or a pyridine nucleus.

In this specification the manner of numbering the substituted positions of the cyanine nucleus of the cyanine dye used in this invention is such that the position of the nitrogen atom is designated as 1.

**DETAILED DESCRIPTION OF THE INVENTION**

Specific examples of the cyanine heterocyclic nucleus of the cyanine dye used in this invention include 20 an oxazoline nucleus, an oxazole nucleus, a benzoxazole nucleus, a naphthoxazole nucleus, a thiazoline nucleus, a thiazole nucleus, a benzothiazole nucleus, a naphthothiazole nucleus, a selenazole nucleus, a benzoselenazole nucleus, a naphthoselenazole nucleus, a 25 2-pyridine nucleus, a 4-pyridine nucleus, a 2-quinoline nucleus, a 4-quinoline nucleus, a 3-isoquinoline nucleus, a 1-isoquinoline nucleus, an imidazole nucleus, a benzimidazole nucleus, an indolene nucleus, an imidazo[4,5-b]quinoxaline nucleus, a pyrrolidine nucleus and the like. The benzene rings of those heterocyclic rings and/or the condensed heterocyclic rings may have substituents. Examples of the substituents are an alkyl group, an aryl group, a hydroxyl group, an alkoxy group, a carboxyl group, an alkoxy carbonyl group, a 30 nitro group, and a halogen atom, with preferred alkyl groups or moieties having 1-20 carbon atoms, preferred alkoxy groups having 1-10 carbon atoms and a preferred aryl group being a phenyl group.

As examples of such cyanine nuclei, there are thiazoles such as thiazole, 4-methylthiazole, 4-phenylthiazole, 4-(p-hydroxyphenyl)thiazole, 5-methylthiazole, 5-phenylthiazole, 5-(o-hydroxyphenyl)thiazole, 4,5-dimethylthiazole and 4,5-diphenylthiazole; benzothiazoles such as benzothiazole, 4-hydroxybenzothiazole, 4-fluorobenzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5,6-dimethylbenzothiazole, 5-bromobenzothiazole, 6-bromobenzothiazole, 5-phenylbenzothiazole, 6-phenylbenzothiazole, 4-phenylbenzothiazole, 4-methoxybenzothiazole, 5-methoxybenzothiazole, 6-methoxybenzothiazole, 7-methoxybenzothiazole, 5-iodobenzothiazole, 6-iodobenzothiazole, 5-ethoxybenzothiazole, 4-ethoxybenzothiazole, 5-ethoxycarbonylbenzothiazole, tetrahydrobenzothiazole, 5-(N,N-dimethylamido)benzothiazole, 5,6-dimethoxybenzothiazole, 5-hydroxybenzothiazole, 6-hydroxybenzothiazole, 5-nitrobenzothiazole and 5-chloro-6-nitrobenzothiazole; naphthothiazoles such as  $\alpha$ -naphthothiazole,  $\beta$ -naphthothiazole,  $\beta,\beta$ -naphthothiazole, 8-methoxy- $\beta$ -naphthothiazole, 5-ethoxy- $\beta$ -naphthothiazole, 7-methoxy- $\alpha$ -naphthothiazole, 8-methoxy- $\alpha$ -naphthothiazole, 5-hydroxy- $\beta$ -naphthothiazole, 7-hydroxy- $\alpha$ -naphthothiazole and 5-ethyl- $\beta$ -naphthothiazole; oxazoles such as oxazole, 4-methyloxazole, 5-methyloxazole, 5-phenyloxazole, 4-(p-hydroxyphenyl)oxazole, 4,5-diphenyloxazole, 4-ethyloxazole,

4,5-dimethyloxazole, 4-phenyloxazole, and 5-(m-hydroxyphenyl)oxazole; benzoxazoles such as benzoxazole, 5-chlorobenzoxazole, 5-methylbenzoxazole, 5-phenylbenzoxazole, 6-methylbenzoxazole, 6-nitrobenzoxazole, 5,6-dimethylbenzoxazole, 4,6-dimethylbenzoxazole, 5-methoxybenzoxazole, 5-ethoxybenzoxazole, 6-chlorobenzoxazole, 6-methoxybenzoxazole, 5-hydroxybenzoxazole and 6-hydroxybenzoxazole; naphthoxazoles such as  $\alpha$ -naphthoxazole,  $\beta,\beta$ -naphthoxazole,  $\beta$ -naphthoxazole (6-hydroxy- $\beta$ -naphthoxazole); selenazoles such as selenazole, 4-methylselenazole, 4-phenylselenazole and 4-(p-hydroxyphenyl) selenazole; benzoselenazoles such as benzoselenazole; 5-chlorobenzoselenazole, 5-methoxybenzoselenazole, 5-hydroxybenzoselenazole and tetrahydrobenzoselenazole; naphthoselenazoles such as  $\alpha$ -naphthoselenazole,  $\beta,\beta$ -naphthoselenazole,  $\beta$ -naphthoselenazole and 7-hydroxy- $\beta$ -naphthoselenazole; thiazolines such as thiazoline, 4-methylthiazoline, and 4-(p-hydroxyphenyl)-thiazoline; 2-quinolines such as 2-quinoline, 3-methyl-2-quinoline, 5-methyl-2-quinoline, 7-methyl-2-quinoline, 8-methyl-2-quinoline, 6-chloro-2-quinoline, 8-chloro-2-quinoline, 8-fluoro-2-quinoline, 6-methoxy-2-quinoline, 6-ethoxy-2-quinoline, 6-hydroxy-2-quinoline, 7-hydroxy-2-quinoline and 8-hydroxy-2-quinoline; 4-quinolines such as 4-quinoline, 5-methoxy-4-quinoline, 6-methoxy-4-quinoline, 7-methoxy-4-quinoline, 8-methoxy-4-quinoline, 6-methyl-4-quinoline, 7-chloro-4-quinoline and 8-trifluoromethyl-4-quinoline; isoquinolines such as isoquinoline, 3-methylisoquinoline, 5-methylisoquinoline, 7-methylisoquinoline, 6-chloroisoquinoline, 6-methoxyisoquinoline and 8-methoxyisoquinoline; 1-

nitroindolenine; 2-pyridines such as pyridine, 4-methylpyridine, 6-methylpyridine, 4,6-dimethylpyridine, 4-butylpyridine, 4-decylpyridine, 4-octadecylpyridine, 4,6-dibutylpyridine, 4-benzylpyridine, 4-phenylpyridine, 4-(p-hydroxyphenyl)pyridine, 4,6-diphenylpyridine, 4,6-dinaphthylpyridine, 4-chloropyridine, 4-bromopyridine, 4,6-dichloropyridine, 4-chloropyridine, 6-bromopyridine, 4-hydroxypyridine, 4-methoxypyridine, 4-ethoxypyridine, 6-methoxypyridine, 6-ethoxypyridine and 4,6-dimethoxypyridine; 4-pyridines such as pyridine, 2-methylpyridine, 2-butylpyridine, 2-decylpyridine, 2-octadecylpyridine, 2,6-dimethylpyridine, 2,6-dibutylpyridine, 2-benzylpyridine, 2-phenylpyridine, 2-(p-hydroxyphenyl)pyridine, 2,6-diphenylpyridine, 2-chloropyridine, 2-bromopyridine, 2,6-dichloropyridine, 2-hydroxypyridine, 2-methoxypyridine, 2-ethoxypyridine and 2,6-dimethoxypyridine; imidazo(4,5-*b*)-quinoxalines such as 1,3-diethylimidazo(4,5-*b*)-quinoxaline, 1,3-diethyl-6-nitroimidazo(4,5-*b*)-quinoxaline, 1,3-diphenylimidazo(4,5-*b*)-quinoxaline, 6-chloro-1,3-diphenylimidazo(4,5-*b*)-quinoxaline, 1,3-diallylimidazo(4,5-*b*)-quinoxaline and 1,3-dicyclohexylimidazo(4,5-*b*)-quinoxaline; oxazine and benzimidazoles such as benzimidazole, 5,6-dichlorobenzimidazole, 1-ethyl-5-nitrobenzimidazole and 1-ethyl-5,6-dichlorobenzimidazole, 1-ethyl-5-methoxycarbonylbenzimidazole, etc.

Among those cayanine heterocyclic nuclei, benzothiazoles, benzoselenazoles, 2-quinolines and 4-quinolines are particularly preferred.

Examples of preferred cyanine dyes used in the present invention can be shown by the following general formulae I and II.

Formula I



Formula II



methylisoquinoline, 6-chloroisoquinoline, 6-methoxyisoquinoline and 8-methoxyisoquinoline; indolenines such as indolenine, 3,3-dimethylindolenine, 5-hydroxy-3,3-dimethylindolenine, 3,3-dimethyl-6-chloroindolenine, 3,3,5-trimethylindolenine and 3,3-dimethyl-5-

65 In the above formulae I and II, R<sub>1</sub> and R<sub>3</sub> each represents an unsubstituted alkyl (C<sub>1</sub>-C<sub>6</sub>)\* group such as a methyl group.

\* the brackets in parentheses indicate preferred carbon atoms in the alkyl moiety

an ethyl group, a propyl group, an isopropyl group, an n-butyl group, an n-pentyl group and an n-hexyl group; a hydroxyalkyl ( $C_1$ – $C_6$ ) group such as a  $\beta$ -hydroxyethyl group and a  $\gamma$ -hydroxypropyl group; an acetoxyalkyl ( $C_1$ – $C_6$ ) group such as a  $\beta$ -acetoxyethyl group, and a  $\gamma$ -acetoxypropyl group; an alkoxyalkyl ( $C_2$ – $C_6$ ) group such as a  $\beta$ -methoxyethyl group and a  $\gamma$ -methoxypropyl group; a carboxyalkyl ( $C_2$ – $C_6$ ) group such as a  $\beta$ -carboxyethyl group, a  $\gamma$ -carboxypropyl group, a  $\gamma$ -carboxybutyl group and a  $\omega$ -carboxypentyl group; an alkoxy-carbonylalkyl ( $C_3$ – $C_6$ ) group such as a  $\beta$ -methoxycarbonylethyl group and a  $\gamma$ -ethoxycarbonylpropyl group; a sulfoalkyl ( $C_1$ – $C_6$ ) group such as a  $\beta$ -sulfoethyl group, a  $\gamma$ -sulfobutyl group and a  $\gamma$ -sulfoethyl group; an aralkyl group such as a benzyl group and a phenethyl group; a sulfoaralkyl group such as a p-sulfophenethyl group; a carboxyaralkyl group such as a p-carboxyphenethyl group; or a vinylmethyl group,  $R_2$  represents a group conventionally known as a substituent for a pyrazolo[1,5-a]benzimidazole compound, such as a hydrogen atom, an alkyl group (e.g., a methyl group, an ethyl group, a propyl group), a benzyl group, a carboxyl group, an alkoxy carbonyl group (e.g., a methoxy carbonyl group and an ethoxycarbonyl group), an amino group, an acylamino group (e.g., an acetylamino group), an aryl group (e.g., a phenyl group and a p-methoxyphenyl group) and an acid amide group,  $L_1$  and  $L_2$  each represents a methine chain such as  $—CH=$  and  $—CR_5=$  (wherein  $R_5$  represents an alkyl group or alkoxyalkyl group such as a methyl group an ethyl group, or an ethoxyethyl group or an aryl group such as a phenyl group), and  $L_1$  and  $R_1$  may combine with each other via a methylene chain, e.g., to form a 5 or 6 membered cyclic ring,  $Z$  represents an atomic group necessary for forming a cyanine heterocyclic nucleus, such as, practically speaking, those mentioned above,  $R_4$  represents a group conventionally known as a substituent for a pyrazolo[1,5-a]benzimidazole compound, such as a halogen atom (e.g., a fluorine atom, a chlorine atom and a bromine atom), a lower alkyl group (e.g., a methyl group and an ethyl group), an alkoxy group (e.g., a methoxy group and an ethoxy group), an aryl group (e.g., a phenyl group), a carboxyl group, an alkoxy carbonyl group (e.g., a methoxycarbonyl group), an acylamino group (e.g., an acetylamino group),  $n$  represents 0 or 1,  $m$  represents 0, 1 or 2,  $p$  represents 1, 2, 3 or 4, and  $X^\ominus$  represents an acid anion such as a chloride ion, a bromide ion, an iodide ion, a thiocyanate ion, a perchloride ion, a p-toluenesulfonate ion, a methylsulfate ion and an ethylsulfate ion.

The cyanine dyes shown by the aforesaid general formula I can be prepared by reacting under heating a compound represented by general formula III

Formula III



wherein  $R_2$ ,  $R_4$ , and  $p$  have the same significance as in the General formula I and a heterocyclic quaternary ammonium salt represented by the general formula IV



wherein  $Y$  represents  $SR'$ ,  $OR''$ , or



(wherein  $R'$  and  $R''$  each represents a methyl group, an ethyl group or a phenyl group) and  $R_1$ ,  $Z$ ,  $L_1$ ,  $L_2$ ,  $n$ ,  $m$ , and  $X^\ominus$  have the same significance as in General formula I in ethanol in the presence of an organic base such as triethylamine.

The cyanine dyes represented by general formula I can also be prepared by reacting a compound represented by general formula V obtained by subjecting the compound of the above-mentioned general formula III to a Vilsmeier reaction

Formula V



wherein  $R_2$ ,  $R_4$ , and  $p$  have the same significance as in general formula I and a heterocyclic quaternary ammonium salt represented by general formula VI



wherein  $R_1$ ,  $L_1$ ,  $L_2$ ,  $X^\ominus$ ,  $Z$ ,  $m$ , and  $n$  have the same significance as in general formula I in acetic anhydride with heating and then treating the product with an alkali. In place of reacting the above reactants in acetic anhydride, both reactants may be reacted in nitrobenzene in the presence of an organic base such as triethylamine, while heating, before the alkali treatment.

The dyes represented by general formula II may be obtained by alkylating a cyanine dye represented by general formula I with an ordinary quaternizing reagent such as dimethyl sulfate, methyl-p-toluenesulfonate, propane sultone, butane sultone and an alkyl halide. In this case, it is possible that the alkylation will occur to the nitrogen atom at the 1-position of the pyrazolo[1,5-a]benzimidazole nucleus or the nitrogen atom at the

4-position thereof, but for the sake of convenience the chemical structure of the dye prepared by the above alkylation is shown by general formula II. It shall be understood, however, that the compound prepared by the above alkylation also includes the compound of the following general formula II'

wherein  $R_1$ ,  $R_2$ ,  $R_3$ ,  $R_4$ ,  $Z$ ,  $L_1$ ,  $L_2$ ,  $n$ ,  $m$ ,  $p$ , and  $X^\ominus$  have the same significance as in the general formula II.

Specific examples of the cyanine dyes used in this invention are illustrated below together with their absorption maximum wave lengths ( $\lambda_{max}^{MeOH}$ ) in methanol solution.



3,925,084

9

10

(4)



(5)



(6)



(7)



3,925,084

11

(8)



12

 $\lambda_{\text{max}}^{\text{MeOH}}$ 554m $\mu$ 

(9)



(10)



(11)



(12)



(13)



(14)



(15)



**15****16**

(16)


 $\lambda_{\text{MeOH}}^{\text{max}}$  540m $\mu$ 

(17)


 $\lambda_{\text{MeOH}}^{\text{max}}$  536m $\mu$ 

(18)


 $\lambda_{\text{MeOH}}^{\text{max}}$  483m $\mu$ 

(19)


 $\lambda_{\text{MeOH}}^{\text{max}}$  510m $\mu$

(20)



(21)



(22)



(23)



3,925,084

**19****20**

(24)



(25)



(26)



(27)



(28)



(29)



( 30 )



(31)



(32)


 $\lambda_{\text{max}}^{\text{MeOH}}$  490 m $\mu$ 

(33)


 $\lambda_{\text{max}}^{\text{MeOH}}$  498 m $\mu$ 

(34)


 $\lambda_{\text{max}}^{\text{MeOH}}$  482 m $\mu$

Some specific examples of synthesizing various dyes used in this invention will now be given.

1. Synthesis of the intermediate [2-methyl-3-dimethylaminomethylene-pyrazolo[1,5-a]benzimidazole (Formula V'):  
Formula III'



A solution prepared by dropwise adding 1 g of phosphorus oxychloride to 20 ml of dimethylformamide while under ice-cooling is added to a solution of 3 g of 2-methylpyrazolo[1,5-a]-benzimidazole in 30 ml of dimethylformamide and the mixture is heated for 1 hour on a warm water bath at atmospheric pressure. The reaction product is cooled, added to water, and the solution is neutralized by adding an aqueous solution of sodium carbonate. The crystals precipitated are recovered by filtration, washed with water, and dried to give 2.4 g of the above intermediate product having a melting point of 216°C.

In the same manner as above, except varying the starting materials, 2-phenyl-3-dimethylaminomethylene-pyrazolo[1,5-a]-benzimidazole is also obtained as crystals melting at 235°C.

2. Synthesis of dye 2:

Dye 2



i. 2 g of 2-acetanilidevinyl-3-ethylbenzothiazolium iodide and 1 g of 2-methylpyrazolo[1,5-a]benzimidazole are refluxed for 1 hour in 50 ml of ethanol on a warm water bath in the presence of 2 ml of triethylamine at atmospheric pressure. After cooling, water is added to the reaction product and then the product is extracted with benzene. After drying the benzene solution over anhydrous sodium sulfate, the solution is concentrated and the reaction product is then separated by means of alumina column chromatography. By recrystallizing the product from ethanol, 0.5 g of the crystals of dye 2 melting at 146°C are obtained.

ii. 3.5 g of 3-ethyl-2-methyl-benzothiazolium-p-toluenesulfonate and 2.3 g of the 2-methyl-3-dimethylaminomethylene-pyrazolo[1,5-a]benzimidazole prepared by the above synthesis of the intermediate are refluxed in 100 ml of acetic anhydride for 2 minutes by heating at atmospheric pressure to conduct the reaction, and then the crystals formed are separated by filtration and dried (acid-addition product of the dye 2). The crystals thus obtained are dissolved by heating in 10 methanol and then a small amount of aqueous sodium hydroxide solution is added to the solution, whereby crystals are formed. When the crystals are recovered by filtration and recrystallized from ethanol, 4 g of dye 2 is obtained.

15. 3. Synthesis of dye 18:

0.5 g of dye 2 is reacted with 1 ml of methyl-p-toluenesulfonate by heating for one minute at atmospheric pressure. After cooling the reaction product, the crystals precipitated are recovered, washed with 20 ether, and dissolved in methanol. Then, an aqueous sodium iodide solution is added to the methanol solution and the crystals precipitated are recovered by filtration, washed with water and dried. When the crystals obtained are recrystallized from a mixture of methanol and chloroform, 0.4 g of dye 18 melting at 274°C. is obtained.

Other dye intermediate products and dyes can easily be prepared in substantially the same manner as above merely by varying the starting materials.

30 Having thus described the synthesis of representative dyes in accordance with this invention, it is appropriate to describe in greater detail certain preferred embodiments of this invention.

It is preferred that the direct positive silver halide emulsion of this invention contain an organic desensitizer.

The organic desensitizer used herein refers to a material having the faculty of catching or trapping free electrons generated in silver halide grains by irradiation 40 and capable of being adsorbed on the silver halide. The organic desensitizer can further be defined as a material having a minimum space electron energy level lower than the electron energy level of the conductive zone of the silver halide grains. It is preferably a compound having a maximum occupied electron energy level lower than the valence electron zone of the silver halide grains. The values of these electron energy levels can be determined, although complicated procedures are required for the measurement.

50 For instance, a practical example of determining the electron energy levels for simple symmetric cyanine dyes is reported by Tani and Kikuchi: "Photographic Science and Engineering"; Vol. 11 (3), 129 (1967) and a practical example of determining the electron energy levels for typical merocyanine dyes is reported by Shiba and Kuboderu; Presentation No. B-12" of the International Congress of Photographic Science, 1970 (Moscow).

It is known that these electron energy levels correspond linearly to the anode polarographic half wave potentials (Eox) and the cathode polarographic half wave potentials (Ered).

Many of such organic desensitizers as can be used in this invention are described in the specifications of U.S. 65 Pat. Nos. 3,023,102; 3,314,796; 2,901,351; and 3,367,779; British Pat. Nos. 723,019; 698,575; 698,576; 834,839; 667,206; 748,681; 796,873; 875,887; 905,237; 907,367; and 940,152; French Pat. Nos. 1,520,824; 1,518,094; 1,518,095; 1,520,819;

1,520,823; 1,520,821; and 1,523,626; Belgian Pat. Nos. 722,457 and 1,523,626; and Japanese Pat. Nos. 13,167/1968 and 14,500/1968.

Any compound as described above can be used as the organic desensitizer(s) in this invention, but particularly useful desensitizers are compounds having a cathode polarographic half wave potential (E<sub>red</sub>) more positive than -1.0 volt represented by general formula VII.

Formula VII



wherein R represents an alkyl group or an allyl group, a represents 1 or 2, and Z, X<sup>-</sup>, and m have the same significance as in general formula I.

Specific examples of R include a methyl group, an ethyl group, a butyl group, a hydroxalkyl group (e.g., a hydroxyethyl group), a carboxyalkyl group (e.g., carboxymethyl group and a 3-carboxypropyl group) and a sulfoalkyl group (e.g., a 2-sulfoethyl group and a 4-sulfobutyl group).

Specific examples of organic desensitizers which can be employed in the present invention are, phenosafranine, pinakryptol yellow, 5-m-nitrobenzylidenerhodanine, 3-ethyl-5-m-nitrobenzylidene rhodanine, 3-ethyl-5-(2,4-dinitrobenzylidene) rhodanine, 5-o-dinitrobenzylidene-3-phenylrhodanine, 1',3-diethyl-6-nitrothio-2'-cyanine.iodine salt, 4-nitro-6-chlorobenzotriazole, 3,3'-diethyl-6,6'-dinitro-9-phenylthiacarbocyanine.iodine salt, 2-(p-dimethylaminophenylminomethyl)benzothiazole.ethoethyl sulfate, crystal violet, 3,3'-diethyl-6,6'-dinitrothiacyarbocyanine.ethyl sulfate, 1',3-diethyl-6-nitrothio-2'-cyanine.iodine salt, 1,3-diamino-5-methylphenazinium chloride, 4-nitro-6-chlorobenzotriazole, 3,3'-di-p-nitrobenzylthiacarbocyanine bromide, 3,3'-di-p-nitrophenylthiacarbocyanine.iodine salt, 3,3'-di-p-nitrophenylthiacarbocyanine 3,3'-dimethyl-9-trifluoromethylthiacarbocyanine.iodine salt, 9-(2,4-dinitrophenylmercapto)3,3'-diethylthiacarbocyanine.iodine salt, bis(4,6-diphenylpyrlyl-2-trimethinecyanine perchlorate, anhydrous 2-p-dimethylaminophenylminomethyl-6-nitro-3-(4-sulfonyl)-benzothiazolium hydroxide, 1-(2-benzothiazoly)-2-(p-dimethylaminostyryl)-4,6-diphenylpyridinium.iodine salt, 1,3-diethyl-5-[1,3-neopentylene-6-(1,3,3-trimethyl-2-indolinylidene)-2,4-hexadienylidene]-2-thiobarbituric acid, 2,3,5-triphenyl-2H-tetrazolium chloride, 2-(4-iodophenyl)-3-(4-nitrophenyl)-5-phenyl-tetrazolium chloride, 1-methyl-8-nitroquinolinium methyl sulfate and 3,6-bis[4-(3-ethyl-2-benzothiazolinylidene)-2-butenylidene]-1,2,4,5-cyclohexanotetraen.

As silver halide emulsions used in this invention, there are illustrated a silver chloride emulsion, a silver bromide emulsion, a silver chlorobromide emulsion, a silver chloroiodide emulsion and a silver chloroiodobromide emulsion.

The grain size of such silver halides can be in the generally used range, but particularly good results are obtained when a silver halide having a mean grain size of 0.05 microns to 1.0 micron is used. Also, the silver halide grains used in this invention can be regular grains or irregular grains, but the invention is applied more effectively when regular silver halide grains are used.

Furthermore, a simple dispersion type silver halide emulsion or a non-simple dispersion type silver halide emulsion can be used in this invention, but the use of a simple dispersion type emulsion is more preferred.

5 In general, silver halide emulsions used for direct positive silver halide photographic materials are classified into the following two types.

The first type is a silver halide emulsion having nuclei capable of trapping free electrons in the silver halide 10 crystals, the surfaces of the silver halide grains of which have been preliminarily fogged chemically. The main feature of the silver halide emulsion of this type is that by the addition of a sensitizing dye or dyes the silver halide emulsion is highly sensitized by the action of 15 spectral sensitization as well as being sensitized in its characteristic absorption region. A silver halide emulsion of this type is required to have its halogen composition adjusted so that the chemical sensitizers or the salts of metals belong to group VIII of the periodic table used for providing free electron trapping nuclei are readily incorporated in the silver halide. Furthermore, by adding an organic desensitizer to the silver halide emulsion, the occurrence of clearance and particularly the occurrence of re-reversal can be prevented. 20 Still further, by adding bromide ions or iodide ions to a silver halide emulsion of this type the maximum density can be increased, the emulsion can be further sensitized and also the occurrence of clearance can be prevented.

25 Emulsions of this type are described in U.S. Pat. Nos. 2,401,051, 2,717,833, 2,976,149 and 3,023,102, British Pat. Nos. 707,704, 1,097,999 and 1,520,822, and French Pat. Nos. 1,523,626, 1,520,817 and 1,520,824.

The second type is a silver halide emulsion which has no free electron trapping nuclei in the silver halide, the 30 surfaces of the silver halide grains of which have been chemically fogged. This type of emulsion has crystal defects as low as possible and comprises regular silver halide crystals having no twinning plane, and is preferably pure silver bromide. While this type of silver halide 35 emulsion does not give direct positive images per se, if an organic desensitizer is adsorbed on the silver halide of the emulsion, direct positive images can be obtained.

Emulsions of this type are described in U.S. Pat. Nos. 3,501,306, 3,501,307, 3,501,310 and 3,531,288, British Pat. Nos. 1,186,717, 1,186,714 and 1,186,716, and French Pat. Nos. 1,520,821, 1,520,817, 1,522,354 and 40 1,520,824.

In the present invention, silver halide emulsions of 45 both types can be employed. In other words, both types of the aforesaid silver halide emulsions can be effectively sensitized by the compound or the cyanine dyes of the present invention.

The silver halide emulsions used in this invention can 50 be fogged by light or chemically. Chemically fogged nuclei are formed by the addition of a reducing organic compound such as a hydrazine derivative, formalin, thiourea dioxide, a polyamine compound, amine borane or methyl dichlorosilane and the like as disclosed in Belgian Pat. Nos. 721,564 and 708,563, U.S. Pat. No. 2,588,982, British Pat. No. 821,251, French Pat. No. 739,755 and Japanese Pat. Publication No. 43-13488.

The fogged nuclei can also be formed, in addition to 55 the aforesaid manner, by the combination of a reducing agent and ions of a metal nobler than silver, such as gold ions, platinum ions or iridium ions or by a combination of such metals and halogen ions, as disclosed in U.S. Pat. Nos. 2,717,833 and 3,023,102, Belgian Pat. Nos. 713,272 and 721,567 and British Pat. No. 707,704.

In the silver halide emulsion of this invention, gelatin is generally used as the protective colloid, and inert gelatin is particularly preferred. However, instead of gelatin a photographically inert gelatin derivative or water-soluble synthetic polymer such as polyvinyl acrylate, polyvinyl alcohol, polyvinyl pyrrolidone, polyvinyl alginate, carboxymethyl cellulose, and hydroxymethyl cellulose may be used, as may mixtures of any such materials.

The direct positive silver halide emulsions of this invention can further contain, if desired, a stabilizer for the fogged nuclei, such as a mercapto compound, a thion compound or a tetraazaindene compound; an agent to prevent the occurrence of clearing (often referred to as uncoloring), such as a stilbene compound or an azine compound; a whitening agent; an ultraviolet absorbant; a hardening agent such as chromium alum, a 2,4-dichloro-s-triazine compound, an aziridine compound, an epoxy compound, a mucohalogenetic acid compound (e.g., halogen formyl maleic acid compound); a wetting agent such as sodium polyalkylene sulfonate or saponin or an anionic surface active agent having a betaine structure; an antiseptic or disinfectant agent; a plasticizer such as polyalkyl acrylate, a copolymer of an alkylacrylate and acrylic acid or a polyalkylene oxide; or a color coupler.

The amount of the dimethine dye depends upon the amount of the silver halide and the surface area of the silver halide grains in the silver halide emulsion, but good results are obtained when the amount is  $1 \times 10^{-6}$  to  $2 \times 10^{-2}$  mol of dye or dyes per mol of silver halide.

These dye(s) are generally added to the silver halide emulsion as a solutions in a solvent miscible with water, such as methanol, ethanol, ethyleneglycol monomethyl ether, methylethyl ketone, acetone and pyridine, as well as water. Upon dissolving the dye(s) in such a solvent, ultrasonic waves may be applied to the system to promote dissolution. Further, the methods used for the sensitization of negative silver halide emulsions such as the method described in Japanese Pat. Nos. 23,389/1959, 27,555/1969, and 22,948/1969; U.S. Pat. Nos. 3,485,634; 3,342,605; and 2,912,343; and German Patent Application (OLS) No. 1,947,935 may also be employed.

It is convenient to add the dyes to the silver halide emulsion just before coating, but they can be added during chemical ripening of the silver halide emulsions or during precipitation of the silver halide(s).

The amount of the organic desensitizer used in the present invention depends upon the kind of desensitizer, but is preferably  $2 \times 10^{-7}$  to  $10^{-1}$  mol per mol of silver halide.

The silver halide emulsions of this invention can be applied to various supports to give photographic elements. The silver halide emulsions of this invention can be applied to one surface or both surfaces of the support and the support may be transparent or opaque. Typical examples of the supports are cellulose nitrate films, cellulose acetate films, polyvinyl acetal films, polystyrene films, polyethylene terephthalate films, other polyester films, glasses, papers, metallic foils and woods. Plastic-laminated papers can also be used as the support. The exact support chosen is not important.

The photographic silver halide material comprising the silver halide emulsion layer of this invention may be processed after exposure in the manner used for prior art direct positive emulsions, e.g., in separate development, fix, stabilization, etc., baths or in a bath having a combination of such processing functions.

The first feature of the present invention is that the direct positive silver halide emulsion is sensitized by at

least one cyanine dye having the pyrazolo[1,5-a]benzimidazole nucleus. In particular, such alkylated cyanine dyes give higher sensitivity to the silver halide emulsion.

The second feature of the present invention is that a direct positive silver halide emulsion having a sharp spectral sensitization maximum is obtained. In other words, the spectral sensitivity curve of the direct positive silver halide emulsion of this invention has such a form that the longer wave length end of it is sharply cut. Therefore, the photographic materials prepared using the direct positive silver halide emulsions of this invention can be easily handled under a safe light.

The third feature of the present invention is that the cyanine dye (or dyes) having the pyrazolo[1,5-a]benzimidazole nucleus used in this invention has the excellent property of not substantially reducing the maximum density of the direct positive silver halide emulsion.

The fourth feature of the present invention is that the direct positive silver halide emulsion of this invention shows substantially no reduction in maximum density during storage.

The novel dimethine dyes used in this invention have such excellent features as mentioned above, and further by using the dimethine dyes together with the aforesaid organic desensitizers, the reversal sensitivity of the silver halide emulsions can further be improved and also direct positive silver halide emulsions showing excellent clearance can be prepared.

The direct positive silver halide emulsions of this invention can, of course, be used for making duplicating photographic materials for lithographic films and hard or high contrast direct positive silver halide photographic materials used for duplicating originals as well as for making duplicating photographic materials for microphotographic films and also comparatively soft direct positive silver halide photographic materials such as duplicating photographic materials for X-ray photographs. The direct positive silver halide emulsion can also be used for making color photographic materials.

The direct positive silver halide emulsions of this invention can be used not only for the case of exposure to light, but also for the case of exposure to electrons, X-rays or gamma rays.

Moreover, the dimethine dyes to be used in this invention can be also used as photographic dyes, such as dyes for light-filtering layers, dyes for anti-irradiation and antihalation, etc.

The invention will now be illustrated in more detail by referring to the following several examples.

All percentages are weight percent, unless otherwise indicated.

#### EXAMPLE 1

The following four solutions were prepared for making silver halide emulsion.

|                                                  |         |  |
|--------------------------------------------------|---------|--|
| First solution:                                  |         |  |
| inert gelatin                                    | 8 g     |  |
| aqueous potassium bromide solution<br>(1 normal) | 5 cc    |  |
| water (60°C)                                     | 500 cc. |  |
| Second solution:                                 |         |  |
| silver nitrate                                   | 100 g   |  |
| water (60°C)                                     | 500 cc. |  |
| Third solution:                                  |         |  |
| potassium bromide                                | 70 g    |  |
| water (60°C)                                     | 150 cc. |  |
| Fourth solution:                                 |         |  |
| inert gelatin                                    | 75 g    |  |
| water                                            | 300 cc. |  |

While maintaining the system at 60°C, the second solution and the third solution were added to the first solution over a 50 minute period and then the mixture was physically ripened for 5 minutes by permitting it to stand at 60°C. Then, 15 cc of a 0.2 normal aqueous potassium iodide solution was added to the ripened mixture and thereafter the pAg of the mixture was adjusted to 6.0 using an aqueous silver nitrate solution. Then, 12 mg hydrazine and 1.0 mg gold chloride were added to the mixture and after adjusting the pH thereof to 10 using aqueous sodium hydroxide solution, the resultant mixture was further ripened for 10 minutes by permitting it to stand at 60°C. The mixture was neutralized using citric acid and then was washed with water. The mixture was melted again and the forth solution indicated above was added thereto to give the silver halide emulsion. The silver halide emulsion thus prepared contained silver halide grains having a mean grain size of about 0.2 microns, the silver halide grains being regular tetragonal system grains having the (100) plane.

A methanol solution of the dimethine dyes as shown in Table 1 was added to the silver halide emulsion prepared above, and after further adding 40 ml/Kg of emulsion of a 4 wt % aqueous solution of saponin, the resultant emulsion was applied to a cellulose triacetate film in a dry thickness of about 5 microns to give a sample photographic material.

The sample was exposed for 1 second through an optical wedge to a tungsten light source of 2854°K, developed in the developer having the following composition for 2 minutes at 20°C., and then fixed in an acid hardening fix solution.

Composition of the developer:

|                                 |          |
|---------------------------------|----------|
| Metol                           | 3.1 g    |
| anhydrous sodium sulfite        | 45 g     |
| hydroquinone                    | 12 g     |
| sodium carbonate (mono-hydrate) | 79 g     |
| potassium bromide               | 2 g      |
| water added to                  | 1 liter. |

At use, the above composition was diluted with water at a 1:1 volume ratio.

By measuring the density of the sample thus processed by means of a P-Type Densitometer (made by Fuji Photo Film Co.), the characteristic curves of the photographic film were obtained. The sensitivity, the maximum optical density (D<sub>max</sub>) and the minimum optical density (D<sub>min</sub>) thus obtained are shown in Table 1. In addition, the sensitivity is shown by the relative value of the reciprocal of the exposure amount necessary for giving a density of (D<sub>max</sub> + D<sub>min</sub>)/2.

Table 1

| Sample | Dye | (mol density*)<br>cc/100 g of<br>emulsion | Sensitivity | D <sub>max</sub> | D <sub>min</sub> |
|--------|-----|-------------------------------------------|-------------|------------------|------------------|
| 1      | —   | —                                         | —           | 2.8              | —                |
| 2      | 4   | (8 × 10 <sup>-2</sup> )                   | 16          | 890              | 2.7              |
| 3      | 19  | (8 × 10 <sup>-2</sup> )                   | 16          | 1320             | 2.8              |
| 4      | 20  | (8 × 10 <sup>-2</sup> )                   | 24          | 100              | 2.8              |
| 5      | 21  | (8 × 10 <sup>-2</sup> )                   | 16          | 159              | 2.8              |
| 6      | 22  | (8 × 10 <sup>-2</sup> )                   | 32          | 4790             | 2.8              |
| 7      | 28  | (8 × 10 <sup>-2</sup> )                   | 16          | 200              | 2.7              |
| 8      | 12  | (8 × 10 <sup>-2</sup> )                   | 16          | 112              | 2.7              |

\*mol density means mols of dye per liter of solution

From the results shown in Table 1, it will be understood that the direct positive silver halide emulsions of this invention have high sensitivity and D<sub>max</sub>, and fur-

ther show good clearance. Also, it will be understood the alkylated dyes among the above-indicated dyes of this invention gave direct positive silver halide emulsions having higher sensitivity (refer to Sample 2 and Sample 3). Furthermore, the dyes used in this example having the quinoline nucleus as the cyanine heterocyclic nucleus gave particularly high sensitivity.

EXAMPLE 2

10 The silver halide emulsion used in this example was prepared in the following manner.

To a first solution prepared by dissolving at 60°C. 10g of inert gelatin and 5 cc of 1 normal aqueous sodium chloride solution in 500 cc of water were added a second solution prepared by dissolving 100 g of silver nitrate in 500 cc of water at 60°C. and a third solution prepared by dissolving 35 g of sodium chloride in 300 cc of water at 60°C., over a 20 minute period with stirring while maintaining the system at 60°C. Thereafter,

15 the mixture was ripened for 50 minutes at 60°C and then a fourth solution prepared by dissolving 14 g of potassium bromide in 200 cc of water at 60°C was added to the mixture with stirring over a 5 minute period. The resultant mixture was then further ripened for 10 minutes at 60°C and, after reducing the temperature to 35°C, the mixture was washed with water. The mixture was heated again, the pH thereof was adjusted to 10, hydrazine and gold chloride were added thereto in the amounts given in Example 1, and the mixture was ripened again for 10 minutes. Thereafter, the pH of the ripened mixture was adjusted to 6.5 using 8 ml of 10 wt % citric acid. Furthermore, a fifth solution prepared by dissolving 75 g of inert gelatin in 300 cc of water was added to the mixture to yield the silver halide emulsion.

20 25 30 35 The mean grain size of the silver halide grains in the silver halide emulsion thus obtained was about 0.15 micron.

32 cc of a methanol solution of pinakryptol yellow in a concentration of  $5 \times 10^{-2}$  mol per liter of solution was 40 added to the silver halide emulsion prepared above and then a methanol solution of a dye as shown in Table 2 was added to the mixture. After further adding thereto suitable amounts of mucochloric acid and saponin as in Example 1, the resultant silver halide emulsion was applied to a cellulose triacetate film in a dry thickness of about 2 microns to give a sample.

45 The sample prepared was exposed\* through an optical wedge to a tungsten light source of 2854°K and developed for 3 minutes at 20°C. in the developer having the following composition.

50 \* exposure time = 1 second

Composition of the developer:

|                          |         |
|--------------------------|---------|
| water (about 30°C)       | 50 cc   |
| anhydrous sodium sulfite | 30 g    |
| p-formaldehyde           | 7.5 g   |
| sodium bisulfite         | 2.2 g   |
| boric acid               | 7.5 g   |
| hydroquinone             | 22.5 g  |
| potassium bromide        | 1.6 g   |
| water added to make      | 1 liter |

55 60 The sample thus developed was then fixed in an acid hardening fix solution.

65 By measuring the density of the sample film by means of a P-Type Densitometer (made by Fuji Photo Film Co.), the characteristic curves were obtained. The results of measuring the sensitivity, D<sub>max</sub>, and D<sub>min</sub> as in Example 1 are shown in Table 2.

Table 2

| Sample | Dye | (mol density*)<br>cc/100 g of<br>emulsion | Sensitivity | D <sub>max</sub> | D <sub>min</sub> |
|--------|-----|-------------------------------------------|-------------|------------------|------------------|
| 1      |     | —                                         | 100         | 3.0              | 0.07             |
| 2      | 18  | (8 × 10 <sup>-2</sup> )                   | 8           | 933              | 2.9              |
| 3      | 20  | (8 × 10 <sup>-2</sup> )                   | 16          | 1620             | 3.0              |
| 4      | 21  | (8 × 10 <sup>-2</sup> )                   | 24          | 251              | 3.0              |
| 5      | 22  | (8 × 10 <sup>-2</sup> )                   | 16          | 282              | 2.9              |
| 6      | 23  | (8 × 10 <sup>-2</sup> )                   | 16          | 282              | 3.0              |
| 7      | 1   | (8 × 10 <sup>-2</sup> )                   | 16          | 132              | 3.0              |

\*same meaning as in Table 1

From the results shown in Table 2, it will be understood that the direct positive silver halide emulsions of this invention have high sensitivity, high D<sub>max</sub>, and good clearance.

While the invention has been described in detail and with reference to specific embodiments thereof, it will be apparent to one skilled in the art that various changes and modifications can be made therein without departing from the spirit and scope thereof.

What we claim is:

1. A fogged direct positive silver halide emulsion containing at least one cyanine dye comprising a pyrazolo[1,5-a]benzimidazole nucleus and a cyanine heterocyclic nucleus, which nuclei may be substituted with substituents as are commonly used in the cyanine dye art, in which the carbon atom at the 3-position of the pyrazolo[1,5-a]benzimidazole nucleus is joined to the 2-position or 4-position of the cyanine heterocyclic nucleus, by a methine chain, the carbon atom being joined to the 4-position, however, only when the cyanine heterocyclic nucleus is a quinoline nucleus or a pyridine nucleus, said cyanine dye being present in a concentration effective to provide high sensitivity, maximum image density and providing substantially no color stains.

tive silver halide emulsion comprises silver halide grains fogged by a reducing agent and a gold compound.

6. A direct positive silver halide emulsion as set forth in claim 1 wherein the silver halide in the silver halide emulsion comprise regular silver halide grains having a mean grain size of 0.05 micron to 1.0 micron.

7. A direct positive silver halide emulsion as set forth in claim 1 wherein said silver halide emulsion further contains at least one organic desensitizer.

8. A direct positive silver halide emulsion as set forth in claim 7 wherein said at least one organic desensitizer is a compound represented by the following formula

15



25

wherein R represents an alkyl group or an allyl group, Z represents an atomic group necessary for forming a cyanine heterocyclic nucleus, X<sup>⊖</sup> represents an acid anion, m represents 0, 1, or 2, and a represents 1 or 2.

30

9. A fogged direct positive silver halide emulsion as set forth in claim 1 wherein said silver halide emulsion as set forth in claim 1 wherein said silver halide emulsion further contains a color coupler for photography.

35

10. A fogged direct positive silver halide emulsion as set forth in claim 1 wherein said cyanine dye is a compound represented by the following formula



55

wherein R<sub>1</sub> represents an alkyl group, a hydroxyalkyl group, and acetoxyalkyl group, an alkoxyalkyl group, a carboxyalkyl group, an alkoxy carbonylalkyl group, a sulfoalkyl group, an aralkyl group, a sulfoaralkyl group, a carboxyalkyl group, or a vinylmethyl group; R<sub>2</sub> represents a hydrogen atom, an alkyl group, a carboxyl group, an alkoxycarbonyl group, an amino group, an acylamino group, an aryl group, or an acid amide group; L<sub>1</sub> and L<sub>2</sub> each represents a methine chain, and L<sub>1</sub> and R<sub>1</sub> may be combined with each other by a methylene chain; Z represents an atomic group necessary for forming a cyanine heterocyclic nucleus; n represent 0 or 1; m represents 0, 1, or 2, and p represents 1, 2, 3, or 4.

60

wherein R<sub>1</sub> represents an alkyl group, a hydroxyalkyl group, and acetoxyalkyl group, an alkoxyalkyl group, a carboxyalkyl group, an alkoxy carbonylalkyl group, a sulfoalkyl group, an aralkyl group, a sulfoaralkyl group, a carboxyalkyl group, or a vinylmethyl group; R<sub>2</sub> represents a hydrogen atom, an alkyl group, a carboxyl group, an alkoxycarbonyl group, an amino group, an acylamino group, an aryl group, or an acid amide group; L<sub>1</sub> and L<sub>2</sub> each represents a methine chain, and L<sub>1</sub> and R<sub>1</sub> may be combined with each other by a methylene chain; Z represents an atomic group necessary for forming a cyanine heterocyclic nucleus; n represent 0 or 1; m represents 0, 1, or 2, and p represents 1, 2, 3, or 4.

65

wherein R<sub>1</sub> represents an alkyl group, a hydroxyalkyl group, and acetoxyalkyl group, an alkoxyalkyl group, a carboxyalkyl group, an alkoxy carbonylalkyl group, a sulfoalkyl group, an aralkyl group, a sulfoaralkyl group, a carboxyalkyl group, or a vinylmethyl group; R<sub>2</sub> represents a hydrogen atom, an alkyl group, a carboxyl group, an alkoxycarbonyl group, an amino group, an acylamino group, an aryl group, or an acid amide group; L<sub>1</sub> and L<sub>2</sub> each represents a methine chain, and L<sub>1</sub> and R<sub>1</sub> may be combined with each other by a methylene chain; Z represents an atomic group necessary for forming a cyanine heterocyclic nucleus; n represent 0 or 1; m represents 0, 1, or 2, and p represents 1, 2, 3, or 4.

2. A fogged direct positive silver halide emulsion as set forth in claim 1 wherein said cyanine dye is an alkylated cyanine dye.

3. A direct positive silver halide emulsion as set forth in claim 1 wherein said cyanine heterocyclic nucleus is a benzathiazole nucleus, a benzaselenazole nucleus, a 2-quinoline nucleus or a 4-quinoline nucleus.

4. A direct positive silver halide emulsion as set forth in claim 1 wherein the silver halide in the direct positive silver halide emulsion comprises chemically fogged silver halide grains.

5. A direct positive silver halide emulsion as set forth in claim 1 wherein the silver halide in the direct posi-

11. A fogged direct positive silver halide emulsion as set forth in claim 1 wherein said cyanine dye is the compound represented by the following formula



wherein R<sub>1</sub> and R<sub>3</sub> each represents an alkyl group, a hydroxyalkyl group, an acetoxyalkyl group, an alkoxyalkyl group, a carboxyalkyl group, an alkoxycarbonylalkyl group, a sulfoalkyl group, an aralkyl group, a sulfoaralkyl group, a carboxyaralkyl group, or a vinylmethyl group; R<sub>2</sub> represents a hydrogen atom, an alkyl group, a carboxyl group, an alkoxycarbonyl group, an amino group, an acylamino group, an aryl group or an acid amide group; L<sub>1</sub> and L<sub>2</sub> each represents a methine chain, and L<sub>1</sub> and R<sub>1</sub> may be combined with each other by a methylene chain; R<sub>4</sub> represents a halogen atom, a lower alkyl group, an alkoxy group, an aryl group, a carboxyl group, an alkoxycarbonyl group or an acylamino group; Z represents an atomic group necessary for forming a cyanine heterocyclic nucleus; X<sup>⊖</sup> represents an acid anion; n represents 0 or 1, m represents 0, 1, or 2; and p represents 1, 2, 3, or 4.

12. A fogged direct positive silver halide photographic material comprising a support having therein a fogged direct positive silver halide emulsion layer, said silver halide emulsion layer containing at least one cyanine dye comprising a pyrazolo[1,5-a]benzimidazole nucleus and a cyanine heterocyclic nucleus, which nuclei may be substituted with substituents as are commonly used in the cyanine dye art, in which the carbon atom at the 3-position of the pyrazolo[1,5-a]benzimidazole nucleus is joined to the 2-position or the 4-position of the cyanine heterocyclic nucleus by a methine chain, said carbon atom being joined to the 4-position, however, only when the cyanine heterocyclic nucleus is a quinoline nucleus or a pyridine nucleus, said cyanine dye being present in a concentration effective to provide high sensitivity, maximum image density and providing substantially no color stains.

13. A fogged direct positive silver halide emulsion as set forth in claim 1 wherein said cyanine heterocyclic nucleus is substituted with a member selected from the group consisting of an alkyl group, an aryl group, an hydroxyl group, an alkoxy group, a carboxyl group, an alkoxycarbonyl group, a nitro group and a halogen atom.

14. A fogged direct positive silver halide emulsion as set forth in claim 13 wherein said alkyl group has 1-20 carbon atoms, said alkoxy group has 1-10 carbon atoms and said aryl group is a phenyl group.

15. A fogged direct positive silver halide emulsion as set forth in claim 14 wherein said pyrazolo[1,5-a]benzimidazole nucleus is substituted with a member se-

lected from the group consisting of an alkyl group, a hydroxyalkyl group, an acetoxyalkyl group, an alkoxyalkyl group, a carboxyalkyl group, an alkoxycarbonyl-

alkyl group, a sulfoalkyl group, an aralkyl group, a sulfoaralkyl group, a carboxyaralkyl group, a vinylmethyl group, hydrogen, a carboxyl group, an alkoxycarbonyl group, an amino group, an acylamino group, an aryl group and an acid amide group.

16. A fogged direct positive silver halide emulsion as set forth in claim 1 wherein in said pyrazolo[1,5-a]benzimidazole nucleus:

the carbon atom at the 2-position thereof is methyl or phenyl substituted;

the benzene ring thereof is unsubstituted;

the nitrogen atom connected to the carbon atom at the 2-position thereof is unsubstituted, methyl substituted or sulfopropyl substituted.

17. A fogged direct positive silver halide emulsion as set forth in claim 13 wherein:

the carbon atom at the 2-position thereof is methyl or phenyl substituted;

the benzene ring thereof is unsubstituted;

the nitrogen atom connected to the carbon atom at the 2-position thereof is unsubstituted, methyl substituted or sulfopropyl substituted.

18. A fogged direct positive silver halide emulsion as set forth in claim 1 wherein said cyanine heterocyclic

nucleus is selected from the group consisting of an oxazoline nucleus, an oxazole nucleus, a benzoxazole nucleus, a naphthoxazole nucleus, a thiazoline nucleus, a thiazole nucleus, a benzothiazole nucleus, a naphthothiazole nucleus, a selenazole nucleus, a benzoselenazole nucleus, a naphthoselenazole nucleus, a 2-pyridine nucleus, a 4-pyridine nucleus, a 2-quinoline nucleus, a 4-quinoline nucleus, a 3-isoquinoline nucleus, a 1-isoquinoline nucleus, an imidazole nucleus, a benzimidazole nucleus, an indolene nucleus, an imidazo[4,5-b]quinoxaline nucleus and a pyrrolidine nucleus.

19. A fogged direct positive silver halide emulsion as set forth in claim 1 wherein the amount of said cyanine dye is  $1 \times 10^{-6}$  to  $2 \times 10^{-2}$  mol of dye or dyes per mol of silver halide.

20. A fogged direct positive silver halide emulsion as set forth in claim 10 wherein the amount of said cyanine dye is  $1 \times 10^{-6}$  to  $2 \times 10^{-2}$  mol of dye or dyes per mol of silver halide.

21. A fogged direct positive silver halide emulsion as set forth in claim 11 wherein the amount of said cyanine dye is  $1 \times 10^{-6}$  to  $2 \times 10^{-2}$  mol of dye or dyes per mol of silver halide.

22. A fogged direct positive silver halide photo-

graphic material as claimed in claim 12 wherein said cyanine dye is a compound represented by the following formula



wherein  $R_1$  represents an alkyl group, a hydroxyalkyl group, an acetoxyalkyl group, an alkoxyalkyl group, a carboxyalkyl group, an alkoxy carbonylalkyl group, a sulfoalkyl group, an aralkyl group, a sulfoaralkyl group, a carboxyaralkyl group, or a vinylmethyl group;  $R_2$  represents a hydrogen atom, an alkyl group, a carboxyl group, an alkoxy carbonyl group, an amino group, an acylamino group, an aryl group, or an acid amide group;  $L_1$  and  $L_2$  each represents a methine chain, and  $L_1$  and  $R_1$  may be combined with each other by a methylene chain;  $Z$  represents an atomic group necessary for forming a cyanine heterocyclic nucleus;  $n$  represents 0 or 1;  $m$  represents 0, 1, or 2, and  $p$  represents 1, 2, 3, or 4.

23. A fogged direct positive silver halide photographic material as claimed in claim 22 wherein the amount of said dye is  $1 \times 10^{-6}$  to  $2 \times 10^{-2}$  mol of dye or dyes per mol of silver halide.

24. A fogged direct positive silver halide photographic material as claimed in claim 12 wherein said cyanine dye is the compound represented by the following formula:



wherein  $R_1$  and  $R_3$  each represents an alkyl group, a hydroxyalkyl group, an acetoxyalkyl group, an alkoxyalkyl group, a carboxyalkyl group, an alkoxy carbonylalkyl group, a sulfoalkyl group, an aralkyl group, a sul-

55 29. A fogged direct positive silver halide photographic material as claimed in claim 24 wherein M is 1 or 2.

\* \* \* \* \*

foaralkyl group, a carboxyaralkyl group, or a vinylmethyl group;  $R_2$  represents a hydrogen atom, an alkyl group, a carboxyl group, an alkoxy carbonyl group, an